

C. F. GAILOR.

WELDED RAIL JOINT.

APPLICATION FILED MAR. 2, 1917. RENEWED APR. 3, 1920.

1,361,379.

Patented Dec. 7, 1920.

Fig. 1.



Fig. 2.



Fig. 3.



Fig. 4.



Fig. 5.



WITNESSES

George Du Bon

John Strohmeier

INVENTOR  
CHESTER F. GAILOR

BY  
Brennan Schenck  
ATTORNEYS

# UNITED STATES PATENT OFFICE.

CHESTER F. GAILOR, OF BROOKLYN, NEW YORK, ASSIGNOR TO ATLANTIC WELDING CORPORATION, OF NEW YORK, N. Y., A CORPORATION OF NEW YORK.

## WELDED RAIL-JOINT.

1,361,379.

Specification of Letters Patent. Patented Dec. 7, 1920.

Application filed March 2, 1917, Serial No. 151,948. Renewed April 3, 1920. Serial No. 370,960.

To all whom it may concern:

Be it known that I, CHESTER F. GAILOR, a citizen of the United States, residing in Brooklyn, Kings county, city and State of New York, have invented certain new and useful Improvements in Welded Rail-Joints, of which the following is a specification.

My invention relates to welded rail joints for railway track systems, particularly to such systems when used in electric railway service. Such joints must not only be of high electrical conductivity but must also be durable and permanently capable of withstanding the shocks and strains of traffic.

My invention can be applied to the rails of any usual track system but will be found especially valuable for forming joints between rails of the girder type.

My invention includes, and I claim accordingly not only an improved method of making a welded rail joint but also the joint itself.

My invention will be better understood by referring to the accompanying drawings in which Figure 1 represents a perspective view of a pair of abutted rail ends connected together by my improved joint; Fig. 2 represents a section taken along the line 2—2 of Fig. 1; Fig. 3 represents the section of Fig. 2 as it would appear immediately after the welding of the fish plates to the rails; Fig. 4 is a view, similar to Fig. 1, showing (very greatly exaggerated) how the rail head and base are deformed if the rail ends are joined by the usual rail joint upon which my invention is an improvement; and Fig. 5 is a section, similar to Fig. 2, taken along the line 5—5 of Fig. 4.

Referring to the drawings, Figs. 1 and 2, showing the finished improved joint of my invention, the reference characters 1, 2 represent the ends of alined and tightly abutting rails and 3, 4 represent fish plates bridging the two rail ends, on opposite sides thereof, and each welded at top and bottom to the head and base of both rails as shown at 5, 5' and 6, 6' respectively. The fish plates preferably have their top and bottom edges beveled or faced off to fit the under side of

the rail head and the upper side of the rail 50 base and have a width such that when in position they are spaced a substantial distance away from the web 7 of the rail. This beveling or facing off is not essential, however, as metal can readily be filled in during 55 the welding operation. Considering the cross section of the finished joint it may be likened to that of a box having sides 3 and 4 and a central partition, the rail web 7, serving as a brace.

Heretofore it has been usual, in joints of this general character, to employ flat fish plates, placing them in position on each side of the rail ends and holding them in such position by means of bolts 8 passing 60 through both plates and the web of the rail. The fish plates would then be welded along their top and bottom edges to both rail ends while the bolts 8 would have their heads 9, at one end, welded to the fish plate and 65 the nuts 10, at the other end, welded both to the fish plates and to the shank of the bolt. Owing to this mode of procedure, the fish plates by reason of the intense heat of welding would expand and, pressing against 70 the more or less inclined surfaces of the rail head and base, slip outwardly away from the web before the operator could succeed in making the weld. The welding being 75 then completed and the joint allowed to cool 80 the equally great contraction would tend to draw the head and the base of the rails together as indicated, on a very greatly exaggerated scale, in Fig. 5 where the dotted lines represent the normal position of the 85 rail head and base before contraction of the fish plates has taken place. The result of this excessive contraction would be a corresponding condition of strain in the two rail ends said strains being a maximum in 90 the regions 11, 11', at the ends of each fish plate and at 12, 12' (shown dotted) in the base and head of the rail respectively near the juncture of said base and head with the rail web. In the course of time, and owing 95 to temperature changes or to the shock of traffic or both, the rail ends have finally yielded to these strains and fracture has

in many cases taken place. As a rule such fractures have been found to take place in the region 11 in the base of the rail just outside the end of each fish plate. As these 5 regions are those having the least strength of all the regions subjected to strain, fracture at these points rather than at others is naturally to be expected. However, under some circumstances, fracture in some of the 10 other indicated regions might also take place.

In practice it is very improbable that the deformation shown in Figs. 4 and 5 would be visible to the naked eye. The position of the parts as shown, however, corresponds in 15 kind to the actual conditions in practice although not in degree and indicates the dangerous strain lines which exist in the usual known type of joint.

In my improved rail joint and mode of 20 making the same I secure all the advantages of the box girder type of welded joint just described without any of the enumerated disadvantages. There are no strained regions in the finished joint and none can develop. There is therefore no tendency to fracture such as has just been described as characteristic of the rail joints heretofore used.

In making my improved joint I use fish 30 plates 3, 4 (Fig. 3) which have been given a slight outward curvature. These fish plates are positioned between head and base of the rail on opposite sides, as usual and the bolts 8 are drawn up sufficiently to hold 35 them in place. They are then welded, as before, along top and bottom edges 5, 6 and 5', 6', to the rail heads and bases respectively. Any expansion in the plates which may take place during the welding operation results 40 either in an increased outward bending of the fish plates or in a slight slip between the fish plate edges and the rail surfaces against which they abut or both. The welding being completed, the nuts 10 are then 45 drawn up upon the bolts 8 so as to draw the central regions of the fish plates toward one another thus straightening the plates. If the initial curvature of the fish plates has been correctly chosen the widening of the 50 plates and consequent forcing apart of rail head and rail base actually taking place or tending to take place and due to the drawing together of the plates by the nuts 10 and bolts 8 will just be equal to the narrowing 55 of the fish plates, and consequent reverse movement or tendency to move of the rail head and rail base, caused by contraction due to cooling. The result will be that when the joint is completed the rail heads and rail 60 bases will be at exactly the same distance apart as they were before the jointing operation was begun and all parts of the rail heads and rail bases will be free from strain and will remain so.

65 Various modifications of detail in both the

joint of my invention and the method of making the same will readily occur to those skilled in the art within the terms and spirit of the following claims. Thus, while I prefer that the entire length of the top and bottom edges of the fish plates be welded fast to the rails, this is not essential and a portion or portions of said edges may be free from welding. So, also, the plates themselves may have shapes other than simple rectangles. Similarly, the essential thing is that the central portions of the fish plates be curved out of the plane which includes the top and bottom edges of the plates and while I prefer the curvature 75 away from the rail web as shown in the drawings, an opposite curvature would serve equally well provided appropriate arrangements for straightening the plates after welding be provided.

Also, instead of bolts 8 and nuts 10 I may use any other usual means for lessening the curvature of the fish plates and for maintaining them permanently in such condition of lessened curvature.

Having described my invention, I claim:—

1. That improvement in the art of making welded rail joints having abutted alined rail ends and a fish plate welded along its top and bottom edges to the head and the 95 base of each rail, which consists in curving the fish plate longitudinally with respect to the rails before welding and in then lessening said curvature after welding.

2. That improvement in the art of making welded rail joints having abutted alined rail ends and a fish plate welded along its top and bottom edges to the head and the 100 base of each rail, which consists in curving the fish plate longitudinally outwardly 105 away from the rails before welding and in then forcing said curved portions, after welding, inwardly toward the rails.

3. That improvement in the art of making welded rail joints having abutted alined rail ends and a fish plate welded along its top and bottom edges to the head and the 110 base of each rail, which consists in curving the fish plate longitudinally outwardly away from the rails before welding, then forcing said curved portions, after welding, 115 inwardly toward the rails and maintaining said portions in said inward positions.

4. The method of making welded rail joints which comprises abutting and alining two rail ends, welding longitudinally curved fish plates along their top and bottom edges to the head and base of both rail ends on opposite sides thereof, and then forcibly and 120 permanently lessening the curvature of said plates.

5. The method of making welded rail joints which comprises abutting and alining two rail ends, welding outwardly and longitudinally curved fish plates along their top 125

70

75

80

85

90

95

100

105

110

115

120

125

130

and bottom edges to the head and base of both rail ends on opposite sides thereof, then drawing and holding said curved portions of the fish plates together by bolts.

- 5 6. A welded rail joint comprising a pair of abutted alined rail ends, fish plates welded along their top and bottom edges to the head and base of each rail on opposite

sides of said rails, and bolts passing through both of said fish plates said plates being in a <sup>10</sup> state of strain tending to curve them longitudinally with respect to the rails and the bolts forcibly resisting such tendency.

In testimony whereof I have hereunto set my hand.

CHESTER F. GAILOR.